

## UNITED STATES PATENT OFFICE

2,277,551

PROCESS OF PRODUCING FAST DYEINGS  
AND THE DYED FIBER OBTAINED THEREBY

Werner Kirst, Konigstein in Taunus, and Erich Fischer, Bad Soden in Taunus, Germany, assignors to General Aniline &amp; Film Corporation, New York, N. Y., a corporation of Delaware

No Drawing. Application November 27, 1940,  
Serial No. 367,377. In Germany July 4, 1939

13 Claims. (Cl. 8—22)

The present invention relates to a process of producing fast dyeings on cellulose fibers or mixtures of cellulose fibers with animal fibers and to the dyed fiber obtained thereby.

A known method of producing fast dyeings on wool consists in applying to the fiber water-soluble azo-dyestuffs containing a grouping capable of forming a metal complex compound, and subsequently treating the dyeings with an agent yielding chromium. In the practice of dyeing cotton only disazo-dyestuffs or polyazo-dyestuffs which contain a salicylic acid grouping or are derivatives of 1,8-dihydroxynaphthalene-4-sulfonic acid, have been after-treated with agents yielding chromium.

Now, we have found that dyeings of very good properties of fastness can be produced on cellulose fibers or mixtures of cellulose fibers with animal fibers, for instance staple fiber from viscose or cuprammonium cellulose and wool, by applying to the fiber a water-soluble azo-dyestuff containing at least one free amino-group and at least once the following grouping:



X being  $\text{NH}_2$ ,  $\text{NHalkyl}$ ,  $\text{N(alkyl)}_2$  or  $\text{OH}$ , and then treating the dyeing obtained with a mixture of cobalt salts and chromates, hydrogen peroxide, alkali-persulfates or alkali perborates.

In general it is not possible to produce on cellulose fibers the same shade as on wool by after-treating with potassium bichromate dyeings obtained by means of ortho-hydroxy-azo-dyestuffs, since a lake is formed only to a limited extent and the dyestuff is removed from the cellulose fiber, especially when mixtures containing animal fiber are being treated. Surprisingly, the same or similar shades as on wool are produced on cellulose fibers by treating the dyeings with a mixture of a cobalt salt and one of the oxidizing agents named above. Removal of the dyestuff from mixed fibers occurs to a much smaller extent so that it is possible, by selection of appropriate methods of dyeing, to produce even dyeings on mixed fibers.

The dyeing is after-treated with the mixture of the metal salts in a neutral or acid solution at a raised temperature. The mixture may contain any chromate or bichromate or any other of the above-named oxidizing agents, and a cobalt salt, as for instance, cobalt sulfate, cobaltous chloride, cobalt acetate or cobalt chromate. By varying the amount of the salt mixture applied and the mixing proportion between the cobalt salt and the oxidizing agent, the shade may be

displaced within certain limits and the velocity of the reaction on the fiber may be influenced.

To the mixture of the oxidizing agents and cobalt salts may be added a dispersing agent, as for instance the condensation product from 1 mol of octodecyl alcohol and 20 mols of ethylene oxide, as well as a protective colloid, whereby the fastness to rubbing of the dyeings is improved. It is also possible to treat the material in the same process of after-treatment with a moth preventive agent, as for instance the product obtained by condensation of 1 mol of benzaldehyde-ortho-sulfonic acid with 2 mols of 2,4-dichloro-1-hydroxybenzene.

15 The after-treatment baths may contain beside the said oxidizing agent and cobalt salt one or more other metal salts, as for instance chromic salts. A chromic salt favorably influences the properties of fastness of the dyeings, especially when the molecule of the dyestuff contains a salicylic acid grouping.

20 The following examples serve to illustrate the invention, but they are not intended to limit it thereto:

25 (1) 1 kilo of a fabric made from 50 parts of wool and 50 parts of staple fiber from viscose is dyed for one hour at 85° C. in a bath containing 70 grams of the sodium salt of the reduced azo-dyestuff 1-amino-2-hydroxy-4-nitrobenzene-3'-aminobenzoyl-3'-aminobenzoyl-2-amino-5-hydroxynaphthalene-7-sulfonic acid, 8 grams of the product obtained by condensation of 1 mol of octodecyl alcohol with 20 mols of ethylene oxide, 80 grams of ammonium sulfate and 600 grams of sodium sulfate in 30,000 cc. of water. The material is then further dyed for one hour at a temperature falling to 70° C., rinsed well and treated for one hour at 90° C.—95° C. in a fresh bath containing 50 grams of a mixture of 20 grams of potassium bichromate, 10 grams of cobaltous chloride and 20 grams of the neutralized condensation product from beta-naphthalenesulfonic acid and formaldehyde, and 20 cc. of acetic acid of 50 per cent strength in 30,000 cc. of water, rinsed again and dried.

30 A black tone-in-tone dyeing of very good properties of fastness is obtained.

(2) 1 kilo of skein of artificial silk staple fiber is dyed for one hour at 70° C.—90° C. in a bath containing in 20,000 cc. of water 60 grams of the sodium salt of the reduced azo-dyestuff 1-amino-2-hydroxy-4-nitrobenzene

acid  
55 2-amino-5-hydroxynaphthalene-7-sulfonic acid  
alkaline

1-amino-2-hydroxy-5-nitrobenzene-3-sulfonic acid and 400 grams of sodium sulfate. The material is then rinsed and treated for 45 minutes at 90° C. in a fresh bath containing 50 grams of a mixture of 20 grams of potassium bichromate, 10 grams of cobaltous chloride and 20 grams of a neutralized condensation product from beta-naphthalenesulfonic acid and formaldehyde, and 20 cc. of acetic acid of 50 per cent strength in 20,000 cc. of water, rinsed again and dried. A black dyeing of very good properties of fastness is obtained.

If the dyeing is produced on a fabric which contains effects of acetate silk, these effects are not dyed.

(3) 1 kilo of mixed yarn consisting of 50 parts of wool and 50 parts of staple fiber from viscose is treated for one hour at 85° C. in a bath containing in 24,000 cc. of water 50 grams of the sodium salt of the reduced azo-dyestuff 1-amino-2-hydroxy-4-nitrobenzene → 2-acetylamino-5-hydroxynaphthalene-7-sulfonic acid, 8 grams of the condensation product from 1 mol of octodecyl alcohol and 20 mols of ethylene oxide, and 80 grams of ammonium sulfate. To this solution are added 600 grams of sodium sulfate, dissolved in 6000 cc. of water, and the material is further dyed for half an hour at about 70° C., rinsed well and treated for one hour at 90° C. to 95° C. in a fresh bath containing in 30,000 cc. of water 60 grams of a mixture of 20 grams of potassium bichromate, 20 grams of cobaltous chloride and 20 grams of the condensation product from 1 mol of octodecyl alcohol and 20 mols of ethylene oxide. A black dyeing of very good properties of fastness, especially of a very good fastness to wet-processing is obtained.

When the dyeing is after-treated in a bath containing in 30,000 cc. of water 60 grams of a mixture of 10 grams of potassium bichromate, 10 grams of chromic fluoride, 20 grams of cobaltous chloride, and 20 grams of the condensation product from 1 mol of octodecyl alcohol and 20 mols of ethylene oxide.

A black dyeing having similar properties of fastness is likewise obtained.

(4) 1 kilo of a mixed fabric consisting of 50 parts of staple fiber from viscose and 50 parts of wool is dyed for one hour at 85° C., in a bath containing in 30,000 cc. of water 70 grams of the sodium salt of the reduced azo-dyestuff 1-amino-2-hydroxy-5-chlorobenzene

acid  
→  
2-amino-5-hydroxynaphthalene-7-sulfonic acid  
alkaline  
←

1-amino-2-hydroxy-3-nitrobenzene-5-sulfonic acid, 10 grams of the condensation product from 1 mol of octodecyl alcohol and 20 mols of ethylene oxide, and 80 grams of ammonium sulfate, 600 grams of sodium sulfate are then added and the fabric is further dyed for about half an hour at a temperature falling to 70° C., rinsed and treated for one hour at 90° C.-95° C. in a bath containing in 30,000 cc. of water 50 grams of a mixture of 20 grams of potassium bichromate, 10 grams of cobaltous chloride and 20 grams of the neutralized condensation product from beta-naphthalene-sulfonic acid and formaldehyde, and 10 cc. of glacial acetic acid.

A blue-black dyeing of very good properties of fastness is obtained.

(5) A mixed fabric from cotton and viscose

artificial silk is impregnated on the foulard at 80° C. to 90° C. with a solution containing per liter 40 grams of the sodium salt of the reduced azo-dyestuff 1-amino-2-hydroxy-4-nitrobenzene

acid  
→  
2-amino-5-hydroxynaphthalene-7-sulfonic acid. The fabric is then dried and padded on the foulard at 80° C.-90° C. with a solution containing per liter of water 24 grams of potassium bichromate, 12 grams of cobaltous chloride and 5 cc. of acetic acid of 50 per cent strength. The material is exposed to the air and then rinsed with hot water, soaped for one minute with a solution containing per liter of water 2 grams of soap and 2 grams of sodium carbonate, rinsed again and dried. A black dyeing of very good properties of fastness is obtained.

(6) 1 kilo of a mixed fabric consisting of 50 parts of wool and 50 parts of staple fiber from viscose is dyed for one hour at 95° C. in a bath containing in 30 liters of water

60 grams of the sodium salt of the reduced azo-dyestuff 1-amino-2-hydroxy-4-nitrobenzene

acid  
→  
1-amino-8-hydroxynaphthalene-4,6-disulfonic acid  
alkaline  
←

1-amino-4-nitrobenzene,  
7.5 grams of the condensation product from 1 mol of octodecylalcohol and 20 mols of ethylene oxide,  
80 grams of ammonium sulfate, and  
600 grams of sodium sulfate.

The fabric is then further treated for half an hour at a temperature falling to 80° C., rinsed and treated for 1 hour at 90° C. in 30 liters of water containing

20 grams of cobaltous chloride,  
20 cc. of acetic acid of 50 per cent strength,  
5 grams of the condensation product from 1 mol of octodecylalcohol and 20 mols of ethylene oxide and  
40 cc. of hydrogen peroxide of 30 per cent strength.

After rinsing and drying, a black dyeing of good fastness properties is obtained. If the dyeing is treated without addition of hydrogen peroxide, the staple fiber is dyed a weaker shade than the wool fiber.

(7) Cotton is padded with a hot solution containing in 1000 cc. of water

55 40 grams of the sodium salt of the reduced azo-dyestuff 1-amino-2-hydroxy-4-nitrobenzene

acid  
→  
2-amino-5-hydroxynaphthalene-7-sulfonic acid,  
10 cc. of caustic soda solution of 34° Bé. and  
50 grams of tragacanth thickening 6:100.

The material is then dried and treated on the foulard at 90° C. with a solution containing in 1000 cc. of water

10 grams of cobaltous chloride,  
12 cc. of acetic acid of 50 per cent strength and  
5 cc. of hydrogen peroxide of 30 per cent strength.

70 It is then rinsed, soaped at boiling temperature with a solution containing per liter of water 3 grams of soap and 2 grams of sodium carbonate, rinsed again and dried.

A blue-black dyeing of very good properties of fastness is obtained.

(8) 1 kilo of a mixture from 50 parts of wool and 50 parts of staple fiber from viscose is dyed for one hour at 85° C. in 30 liters of water containing—

60 grams of the sodium salt of the reduced azo-dyestuff 1-amino-2-hydroxy-4-nitrobenzene-5-sulfonic acid-3'-aminobenzoyl-3'-aminobenzoyl-2-amino-5-hydroxynaphthalene-7-sulfonic acid,

5 grams of the condensation product from 1 mol of octodecylalcohol and 20 mols of ethylene oxide,

80 grams of ammonium sulfate and 600 grams of sodium sulfate.

The material is then further treated for about 3/4 hour at a temperature falling to 70° C. and rinsed. The Bordeaux-red dyeing thus obtained is after-treated for 3/4 hour at 90° C.-95° C. in a bath containing in 30 liters of water

20 cc. of hydrogen peroxide of 30 per cent strength,

30 cc. of acetic acid of 30 per cent strength and 20 grams of cobaltous chloride.

A dark-violet tone-in-tone dyeing of very good properties of fastness is obtained.

(9) 1 kilo of staple fiber from viscose is dyed for one hour at about 90° C. in a bath containing in 20 liters of water

50 grams of the sodium salt of the reduced azo-dyestuff 1-amino-2-hydroxy-4-nitrobenzene

acid

2-amino-5-hydroxynaphthalene-7-sulfonic acid

alkaline

1-amino-2-hydroxy-5-nitrobenzene-3-sulfonic acid and

400 grams of sodium sulfate.

The material is then rinsed and treated for 3/4 hour at 90° C. in a bath containing in 30 liters of water

20 grams of cobaltous chloride,

30 cc. of acetic acid of 30 per cent strength and

20 cc. of hydrogen peroxide of 30 per cent strength.

A black dyeing of very good properties of fastness is obtained.

If in the foregoing example instead of the azo-dyestuff named therein 50 grams of the sodium salt of the reduced azo-dyestuff 1-amino-2-hydroxy-4-nitrobenzene

alkaline

2-amino-5-hydroxynaphthalene-7-sulfonic acid or 50 grams of the sodium salt of the reduced azo-dyestuff 1-amino-2-hydroxy-5-nitrobenzene-4'-amino-C-phenyl-1,2-(N)-imidazolo-5-hydroxynaphthalene-7-sulfonic acid are used, there are likewise obtained black dyeings of very good properties of fastness.

(10) The cotton goods padded as indicated in Example 7 with the hot solution of the dyestuff and dried are padded at 90° C. on the foulard with a solution containing in 1000 cc. of water

5 grams of cobaltous chloride,

30 grams of sodium persulfate and

12 cc. of acetic acid of 50 per cent strength.

The material is then rinsed, soaped, rinsed again and dried.

A blue-black dyeing of very good properties of fastness is obtained.

(11) The cotton goods impregnated with the dyestuff-solution as indicated in Example 7 are dried and padded at 90° C. with a solution containing in 1000 cc. of water

5 grams of cobaltous chloride,  
15 grams of sodium perborate and  
12 cc. of acetic acid of 50 per cent strength.

The material is then rinsed, soaped and dried.

10 A blue-black dyeing of very good properties of fastness is obtained.

(12) 1 kilo of staple fiber from viscose is dyed for one hour at 70° C.-80° C. in a bath containing in 20 liters of water

15 60 grams of the sodium salt of the reduced azo-dyestuff 1-amino-3-nitrobenzene

acid

20 2-amino-5-hydroxynaphthalene-7-sulfonic acid

alkaline

1-amino-2-hydroxy-5-nitrobenzene-3-sulfonic acid,

25 20 grams of sodium carbonate and  
400 grams of sodium sulfate.

The material is then rinsed and treated for 3/4 hour at 80° C.-90° C. in a bath containing in 30 liters of water

20 grams of cobaltous chloride,  
20 cc. of hydrogen peroxide of 30 per cent strength and

30 20 cc. of acetic acid of 50 per cent strength.

After rinsing a black dyeing of good properties of fastness is obtained.

(13) 1 kilo of a mixed fabric consisting of 50 parts of wool and 50 parts of staple fiber from viscose is dyed for one hour at about 80° C. in a bath containing in 30,000 cc. of water

35 80 grams of the sodium salt of the reduced azo-dyestuff 1-amino-2-hydroxy-4-nitrobenzene

alkaline

1 amino-8-hydroxynaphthalene-4,6-disulfonic acid,

40 80 grams of ammonium sulfate and  
600 grams of sodium sulfate.

The fabric is then further dyed for 1/2 hour at a temperature falling to about 65° C.-70° C., rinsed and treated for one hour near boiling temperature in a bath containing in 30 liters of water

20 grams of cobaltous chloride,  
40 cc. of hydrogen peroxide of 30 per cent strength, and

45 60 30 cc. of acetic acid of 30 per cent strength.

It is then rinsed and dried.

A black dyeing of very good properties of fastness is obtained.

(14) If in Example 13 the dyestuff used therein is replaced by 80 grams of the sodium salt of the reduced azo-dyestuff 1-amino-2-hydroxy-4-nitro-5-chlorobenzene

alkaline

50 2-amino-8-hydroxynaphthalene-6-sulfonic acid, a black dyeing of very good properties of fastness is obtained.

(15) If in Example 6 instead of the dyestuff described therein 60 grams of the sodium salt of

the reduced azo-dyestuff 1-amino-4-nitrobenzene-2-carboxylic acid



1-amino-2-hydroxy-4-nitrobenzene are used, a black dyeing of very good properties of fastness is obtained.

The following table indicates the shades of a number of other dyeings obtainable by this invention.

| Parent dyestuff                                | Shade of the dyeing, treated with a mixture of potassium bichromate and cobaltous chloride, on mixtures of wool and artificial silk staple fiber (50:50) |
|------------------------------------------------|----------------------------------------------------------------------------------------------------------------------------------------------------------|
| 1. 1-amino-2-hydroxy-4-nitro-benzene           | Grey.                                                                                                                                                    |
| 2. 1-amino-2-hydroxy-5-chlorobenzene           | Grey.                                                                                                                                                    |
| 3. 1-amino-2-hydroxy-4-nitrobenzene            | Grey.                                                                                                                                                    |
| 4. 1-amino-2-hydroxy-4-nitrobenzene            | Grey.                                                                                                                                                    |
| 5. 1-amino-2-hydroxy-4-nitrobenzene            | Black.                                                                                                                                                   |
| 6. 1-amino-2-hydroxy-4-nitrobenzene            | Violet-brown.                                                                                                                                            |
| 7. 1-amino-2-hydroxy-5-nitrobenzene            | Dark violet.                                                                                                                                             |
| 8. 1-amino-2-hydroxy-4-nitrobenzene            | Black.                                                                                                                                                   |
| 9. 1-amino-2-hydroxy-4-nitrobenzene            | Black.                                                                                                                                                   |
| 10. 1-amino-2-hydroxy-4-nitrobenzene           | Black.                                                                                                                                                   |
| 11. 1-amino-2-hydroxy-4-nitrobenzene           | Black.                                                                                                                                                   |
| 12. 1-amino-2-hydroxy-4-nitrobenzene           | Black.                                                                                                                                                   |
| 13. 1-amino-4-hydroxybenzene-3-carboxylic acid | Violet-brown.                                                                                                                                            |
| 14. 1-amino-2-hydroxy-4-nitrobenzene           | Black.                                                                                                                                                   |
| 15. 1-amino-2-hydroxy-4-nitrobenzene           | Black.                                                                                                                                                   |
| 16. 1-amino-2-hydroxy-4-nitrobenzene           | Black.                                                                                                                                                   |
| 17. 1-amino-2-hydroxy-4-nitrobenzene           | Black.                                                                                                                                                   |
| 18. 1-amino-2-hydroxy-4-nitrobenzene           | Olive.                                                                                                                                                   |
| 19. 1-amino-2-hydroxy-4-nitrobenzene           | Black-violet.                                                                                                                                            |
| 20. 1-amino-2-hydroxy-3-chlorobenzene          | Blue-black.                                                                                                                                              |
| 21. 1-amino-2-hydroxy-4-nitrobenzene           | Reddish black.                                                                                                                                           |
| 22. 1-amino-2-hydroxy-4-nitrobenzene           | Grey.                                                                                                                                                    |
| 23. 1-amino-2-hydroxy-3-nitrobenzene           | Currant.                                                                                                                                                 |
| 24. 1-amino-2-hydroxy-4-nitrobenzene           | Grey.                                                                                                                                                    |
| 25. 1-amino-2-hydroxy-4-nitrobenzene           | Grey-brown.                                                                                                                                              |
| 26. 1-amino-2-hydroxy-5-nitrobenzene           | Black-blue.                                                                                                                                              |
| 27. 1-amino-2-hydroxy-4-nitrobenzene           | Black.                                                                                                                                                   |
| 28. 1-amino-2-hydroxy-4-nitrobenzene           | Black-violet.                                                                                                                                            |
| 29. 1-amino-2-hydroxy-4-nitrobenzene           | Grey.                                                                                                                                                    |
| 30. 1-amino-2-hydroxy-5-nitrobenzene           | Garnet.                                                                                                                                                  |
| 31. 1-amino-2-hydroxy-4-nitrobenzene           | Grey.                                                                                                                                                    |
| 32. 1-amino-2-hydroxy-5-nitrobenzene           | Currant.                                                                                                                                                 |
| 33. 1-amino-2-hydroxy-4-nitrobenzene           | Grey.                                                                                                                                                    |
| 34. 1-amino-2-hydroxy-3-nitrobenzene           | Currant.                                                                                                                                                 |
| 35. 1-amino-4-nitrobenzene                     | Black.                                                                                                                                                   |
| 36. 1-amino-4-nitrobenzene                     | Reddish black.                                                                                                                                           |

## Parent dyestuff

Shade of the dyeing, treated with a mixture of potassium bichromate and cobaltous chloride, on mixtures of wool and artificial silk staple fiber (50:50)

|                                                      |          |                                                                                                         |          |               |
|------------------------------------------------------|----------|---------------------------------------------------------------------------------------------------------|----------|---------------|
| 37. 1-amino-2-hydroxy-5-nitrobenzene-3-sulfonic acid | acid     | 4'-aminobenzoyl-4'-aminobenzoyl-2-amino-5-hydroxynaphthalene-7-sulfonic acid.                           | alkaline | Currant.      |
| 38. 1-amino-2-hydroxybenzene-5-sulfonic acid         | acid     | 1-(2',3'-hydroxynaphthoylamino)-4-aminobenzene                                                          | alkaline | Dark violet.  |
| 39. 1-amino-2-hydroxy-3-nitrobenzene-5-sulfonic acid | acid     | 4'-aminobenzoyl-4'-aminobenzoyl-2-amino-5-hydroxynaphthalene-7-sulfonic acid, reduced.                  | alkaline | Dark currant. |
| 40. 1-amino-2-hydroxy-3-nitrobenzene-5-sulfonic acid | acid     | 3'-aminobenzoyl-3'-aminobenzoyl-2-amino-5-hydroxynaphthalene-7-sulfonic acid, reduced.                  | alkaline | Dark violet.  |
| 41. 1-amino-2-hydroxy-4-nitrobenzene                 | acid     | 2-amino-5-hydroxynaphthalene-7-sulfonic acid                                                            | alkaline | Violet-brown. |
| 42. 1-amino-2-hydroxy-5-nitrobenzene-3-sulfonic acid | acid     | 4'-aminobenzoyl-4'-aminobenzoyl-2-amino-5-hydroxynaphthalene-7-sulfonic acid, reduced.                  | alkaline | Violet-brown. |
| 43. 2 mols of 1-amino-2-hydroxy-5-nitrobenzene       | acid     | 4,4'-bis-[5-oxo-3-methyl-Δ <sup>2</sup> -pyrazolinyl-(1)]-stilbene-2,2'-disulfonic acid, reduced.       | alkaline | Orange-brown. |
| 44. 1-amino-3-nitrobenzene                           | acid     | 2-amino-5-hydroxynaphthalene-7-sulfonic acid                                                            | alkaline | Black.        |
| 45. 1-amino-2-hydroxy-4-nitrobenzene-5-sulfonic acid | acid     | benzoyl-4'-aminobenzoyl-2-amino-5-hydroxynaphthalene-7-sulfonic acid, reduced.                          | alkaline | Dark violet.  |
| 46. 1-amino-2-hydroxy-4-nitrobenzene-5-sulfonic acid | acid     | 4"-amino-benzoyl-4'-aminobenzoyl-2-amino-5-hydroxynaphthalene-7-sulfonic acid, reduced.                 | alkaline | Dark currant. |
| 47. 1-amino-2-hydroxy-4-nitrobenzene                 | acid     | 1-amino-8-hydroxynaphthalene-4,6-disulfonic acid                                                        | alkaline | Black.        |
| 48. 1-amino-4-nitrobenzene-2-carboxylic acid         | acid     | 2-amino-5-hydroxynaphthalene-7-sulfonic acid                                                            | alkaline | Black.        |
| 49. 1-amino-2-hydroxy-4-nitrobenzene                 | alkaline | 2-amino-8-hydroxynaphthalene-6-sulfonic acid, reduced.                                                  | alkaline | Black.        |
| 50. 1-amino-2-hydroxy-4-nitrobenzene                 | alkaline | 1-amino-8-hydroxynaphthalene-4,6-disulfonic acid, reduced.                                              | alkaline | Blue-grey.    |
| 51. 1-amino-2-hydroxy-4-nitrobenzene                 | alkaline | 2,5-dihydroxynaphthalene-7-sulfonic acid, reduced.                                                      | alkaline | Black.        |
| 52. 1-amino-2-hydroxy-4-nitro-5-chlorobenzene        | alkaline | 2-amino-8-hydroxynaphthalene-6-sulfonic acid, reduced.                                                  | alkaline | Black.        |
| 53. 1-amino-2-hydroxy-3,5-dinitrobenzene             | alkaline | 2-amino-5-hydroxynaphthalene-7-sulfonic acid, reduced.                                                  | alkaline | Black.        |
| 54. 1-amino-2-hydroxy-3,5-dinitrobenzene             | alkaline | 2-amino-8-hydroxynaphthalene-6-sulfonic acid, reduced.                                                  | alkaline | Black.        |
| 55. 1-amino-2-hydroxy-3,5-dinitrobenzene             | alkaline | 3'-aminobenzoyl-2-amino-5-hydroxynaphthalene-7-sulfonic acid, reduced.                                  | alkaline | Black.        |
| 56. 1-amino-2-hydroxy-4-nitrobenzene                 | alkaline | 1-amino-8-hydroxynaphthalene-3,6-disulfonic acid, reduced.                                              | alkaline | Grey.         |
| 57. 1-amino-2-hydroxy-4-nitro-5-chlorobenzene        | alkaline | 2-amino-5-hydroxynaphthalene-7-sulfonic acid, reduced.                                                  | alkaline | Black.        |
| 58. 1-amino-2-hydroxy-4-nitrobenzene                 | alkaline | 4"-amino-benzoyl-4'-aminobenzoyl-2-amino-8-hydroxynaphthalene-6-sulfonic acid, reduced.                 | alkaline | Black.        |
| 59. 1-amino-2-hydroxy-4-nitrobenzene                 | alkaline | 2-(N-methyl-4'-hydroxy-5'-carboxy-phenyl-sulfonyl-amino)-8-hydroxynaphthalene-6-sulfonic acid, reduced. | acid     | Grey.         |
| 60. 1-amino-2-hydroxy-4-nitrobenzene                 | alkaline | 1-amino-8-hydroxynaphthalene-4-sulfonic acid                                                            | acid     | Olive-brown.  |
| 61. 1-amino-2-hydroxy-5-nitrobenzene-3-sulfonic acid | alkaline | 2-amino-5-hydroxynaphthalene-7-sulfonic acid,                                                           | alkaline | Dark blue.    |
| 62. 1-amino-2-hydroxy-4-nitrobenzene                 | alkaline | 4'-aminobenzoyl-2-amino-5-hydroxynaphthalene-7-sulfonic acid                                            | acid     | Currant.      |
| 63. 1-amino-2-hydroxy-4-nitrobenzene                 | alkaline | 2-amino-5-hydroxynaphthalene-7-sulfonic acid                                                            | alkaline | Black.        |
| 64. 1-amino-2-hydroxy-4-nitrobenzene                 | alkaline | C-phenyl-1,2-(N)-imidazo-5-hydroxynaphthalene-7-sulfonic acid, reduced.                                 | alkaline | Grey.         |
| 65. 1-amino-2-hydroxy-4-nitro-5-chlorobenzene        | alkaline | 2-amino-5-hydroxynaphthalene-7-sulfonic acid, reduced.                                                  | acid     | Grey.         |
| 66. 1-amino-2-hydroxy-3,5-dinitrobenzene             | acid     | 1-amino-8-hydroxynaphthalene-4-sulfonic acid, reduced.                                                  | acid     | Olive.        |
| 67. 1-amino-2-hydroxy-4-nitrobenzene                 | alkaline | 2-amino-8-hydroxynaphthalene-6-sulfonic acid, reduced.                                                  | acid     | Black.        |



(obtainable by coupling 1 mol of the bispyrazolone from 4,4'-bishydrazino-diphenyl-2,2'-disulfonic acid and aceto-acetic ester with 1 mol of diazotized 1-amino-2-hydroxy-4-nitrobenzene and 1 mol of diazotized 4-amino-4'-hydroxy-1,1'-azobenzene-3'-carboxylic acid and subsequently reducing the nitro-group to the amino-group).

|                                      |      |                                                                    |          |          |
|--------------------------------------|------|--------------------------------------------------------------------|----------|----------|
| 69. 1-amino-2-hydroxy-4-nitrobenzene | acid | 2-amino-5-hydroxynaphthalene-7-sulfonic acid                       | alkaline | Currant. |
| 70. 1-amino-2-hydroxy-4-nitrobenzene | acid | 5,5'-dihydroxy-2,2'-dinaphthylamine-7,7'-disulfonic acid, reduced. | alkaline | Grey.    |

We claim:

1. A process of producing fast dyeings on fibrous material of the group consisting of cellulose fibers and mixtures of cellulose fibers with animal fibers which comprises applying to the fiber an alkali metal salt of a water-soluble azo-

dyestuff containing at least one free amino-group and at least once the following grouping:



wherein X stands for a member of the group consisting of  $\text{NH}_2$ ,  $\text{NH.alkyl}$ ,  $\text{N(alkyl)}_2$  and  $\text{OH}$ , and then aftertreating the dyeing obtained with a mixture of a cobalt salt and an oxidizing agent of the group consisting of chromates, hydrogen peroxide, alkali persulfates and alkali perborates.

2. A process of producing fast dyeings on fibrous material of the group consisting of cellulose fibers and mixtures of cellulose fibers with animal fibers which comprises applying to the fiber an alkali metal salt of a water-soluble azo-dyestuff containing at least one free amino-group and at least once the following grouping:



wherein X stands for a member of the group consisting of  $\text{NH}_2$ ,  $\text{NH.alkyl}$ ,  $\text{N(alkyl)}_2$  and  $\text{OH}$ , and then aftertreating the dyeing obtained with a mixture of a cobalt salt and a chromate.

3. A process of producing fast black dyeings on fibrous material of the group consisting of cellulose fibers and mixtures of cellulose fibers with animal fibers which comprises applying to the fiber an alkali metal salt of a water-soluble azo-dyestuff of the following constitution:



and then after-treating the dyeing obtained with a mixture of a cobalt salt and a chromate.

4. A process of producing fast black dyeings on fibrous material of the group consisting of cellulose fibers and mixtures of cellulose fibers with animal fibers which comprises applying to the fiber an alkali metal salt of a water-soluble azo-dyestuff of the following constitution:



and then after-treating the dyeing obtained with a mixture of cobaltous chloride and potassium bichromate.

5. A process of producing fast black dyeings on fibrous material of the group consisting of cellulose fibers and mixtures of cellulose fibers with animal fibers which comprises applying to the fiber an alkali metal salt of a water-soluble azo-dyestuff of the following constitution:



and then aftertreating the dyeing obtained with a mixture of a cobalt salt and a chromate.

6. A process of producing fast black dyeings on fibrous material of the group consisting of cellulose fibers and mixtures of cellulose fibers with animal fibers which comprises applying to

the fiber an alkali metal salt of a water-soluble azo-dyestuff of the following constitution:



and then aftertreating the dyeing obtained with a mixture of cobaltous chloride and potassium bichromate.

15. 7. A process of producing fast blue-black dyeings on fibrous material of the group consisting of cellulose fibers and mixtures of cellulose fibers with animal fibers which comprises applying to the fiber an alkali metal salt of a water-soluble azo-dyestuff of the following constitution:



and then aftertreating the dyeing obtained with a mixture of a cobalt salt and a chromate.

8. A process of producing fast blue-black dyeings on fibrous material of the group consisting of cellulose fibers and mixtures of cellulose fibers with animal fibers which comprises applying to the fiber an alkali metal salt of a water-soluble azo-dyestuff of the following constitution:



50 and then aftertreating the dyeing obtained with a mixture of cobaltous chloride and potassium bichromate.

9. Fibrous material of the group consisting of cellulose fibers and mixtures of cellulose fibers with animal fibers dyed with a water-soluble azo-dyestuff by the process claimed in claim 1.

10. Fibrous material of the group consisting of cellulose fibers and mixtures of cellulose fibers with animal fibers dyed with a water-soluble azo-dyestuff by the process claimed in claim 3.

11. Fibrous material of the group consisting of cellulose fibers and mixtures of cellulose fibers with animal fibers dyed with a water-soluble azo-dyestuff by the process claimed in claim 5.

12. Fibrous material of the group consisting of cellulose fibers and mixtures of cellulose fibers with animal fibers dyed with a water-soluble azo-dyestuff by the process claimed in claim 7.

13. Fibrous material of the group consisting of cellulose fibers and mixtures of cellulose fibers with animal fibers dyed with a water-soluble azo-dyestuff by the process claimed in claim 8.

WERNER KIRST.  
ERICH FISCHER.